

# UNITED STATES PATENT OFFICE.

CHARLES SCHWARTZ, OF VILLEURBANNE, FRANCE, ASSIGNOR TO SOCIETE GILLET & FILS, OF LYON, RHÔNE, FRANCE, A CORPORATION OF FRANCE.

## PROCESS FOR THE TREATMENT OF VEGETABLE FIBERS.

1,384,677.

Specification of Letters Patent. Patented July 12, 1921.

No Drawing.

Application filed December 9, 1919. Serial No. 343,578.

To all whom it may concern:

Be it known that I, CHARLES SCHWARTZ, a citizen of the Republic of France, and a resident of Villeurbanne, Department of 5 Rhône, France, have invented a new and useful Process for the Treatment of Vegetable Fibers, of which the following is a specification.

This invention relates to a process for 10 treating vegetable fibers, with a view more especially to imparting to them the character of wool, both physically, as to feel, appearance and caloric quality, and chemically, as regards affinity and absorbent capacity for dyestuffs.

In my prior patent applications Nos. 343, 576 and 343,577 of even date herewith, I have described certain processes for treating vegetable fibers of all kinds and in all 20 forms, designed to impart to these fibers the character of wool; the said processes consist in precipitating upon these fibers the products resulting from the action of concentrated nitric acid, preferably of a concentration equal to or higher than 65 per cent., upon cellulose or cellulosic compounds in the one case and starch or amylaceous substances in the other case, this precipitation being effected either by washing with water 25 or by treatment with dilute solutions of acids, bases or salts, followed by washing with water.

It has now been found that the wool-character can also be imparted to vegetable fibers 35 by treating them at the ordinary temperature with concentrated nitric acid, preferably of a concentration equal to or higher than 65 per cent., and removing the acid by washing.

40 This process is likewise applicable to vegetable fibers of all kinds and in all forms, and the raw state or bleached, and whether mercerized or not, at any state whatever in the operations to which they are subjected in the textile industry, and whether they are in the mass, or in the state of lap, cops, card-ends, twistings, yarns or fabrics.

There is produced by this treatment, without however arriving at the same results as 50 those obtained by the processes described in my above mentioned patent applications, a considerable improvement of the vegetable fibers, while obtaining a great simplification in the method of operation; on the other

hand this treatment communicates to the 55 vegetable fibers the character of wool to a degree at least equal to that acquired in the Heberlein process, consisting in passing the fabrics, previously mercerized in alkali, into strong sulfuric acid.

60 The process of this invention presents the following advantages: the time of immersion is not very definitely limited, and the structure of the fabric remains unchanged during the operation; the textile remains 65 strong and may be pressed out at once and washed, contrary to what is the case in the Heberlein process mentioned above, wherein in the reaction is limited to some seconds 70 and cannot be extended without serious drawbacks. Moreover if the fabric is mercerized in alkali and treated with sulfuric acid, it gives rise to a gelatinous mass which cannot be pressed out without being damaged. It is to be noted that the fabric 75 treated according to the process forming the subject of the present application is closer in texture and more fleecy than in the case of the sulfuric acid process; lastly, contrary to what happens in the latter case, the weight 80 of the textile is not only undiminished, but presents an increase by reason of the absorption of nitrogen.

The process according to this invention 85 offers the further advantage of allowing the complete recovery of the nitric acid employed.

This process may be utilized to produce 90 print-effects upon fabrics, either by direct means or by the use of reserves.

The process of the invention may be carried out in the following manner:

The textile material, in the form of fabric, or yarn for example, is steeped in a 95 large excess of concentrated nitric acid, in which it floats freely without any tension, until the reaction is terminated; then it is squeezed or dried out and washed. The time of contact depends upon the concentration of the acid and the quality of the textile material, especially its porosity and absorbent capacity. For example, one minute will be sufficient soaking for ordinary plain fabrics, in 75 per cent. nitric acid; two minutes for ordinary calicoes in 72 per cent. 100 acid; five minutes for fine Egyptian-cotton batistes in 65 per cent. acid.

105 This treatment in nitric acid may be pro-

longed up to five, ten or thirty minutes respectively, without harm as to the final result, on condition that the temperature does not exceed 20° C.; this fact is of great importance in manufacture on a large scale, where it is always necessary to take account of the possibility of stoppages or other causes bringing the apparatus to a standstill for a time.

10 For practical reasons, the temperature of the acid is maintained at a comparatively low temperature, in particular to avoid the evolution of acid vapors, but it is possible to reach 25° C. without risk to the material under treatment.

With nitric acid of a concentration between 65 per cent. and 75 per cent., it is possible without inconvenience and at the ordinary temperature, to allow the action 20 of the nitric acid upon the fiber to be prolonged. When on the other hand this concentration-limit of 75 per cent. is exceeded, it is necessary to insure that the nitric acid acts upon the fiber only for a very short 25 time, some few minutes for example, this time varying inversely in proportion to the concentration of the acid.

Having now particularly described and ascertained the nature of my said invention

and in what manner same is to be performed, I declare what I claim is:—

1. A process for the treatment of vegetable fibers with a view to impart to them the character of wool, both physically, as to feel, appearance and caloric quality, and 35 chemically, as regards their affinity and absorbent capacity for dyestuffs, said process comprising treating the vegetable fiber at the ordinary temperature with concentrated nitric acid and removing the acid by washing. 40

2. A process for the treatment of vegetable fibers with a view to impart to them the character of wool, both physically, as to feel, appearance and caloric quality, and 45 chemically, as regards their affinity and absorbent capacity for dyestuffs, this process consisting in treating these fibers at the ordinary temperature with nitric acid of a concentration of at least 65%, and in removing the acid by washing. 50

In testimony whereof I have signed my name to this specification.

CHARLES SCHWARTZ.

Witnesses:

PHILIPPE DESGRANGES,  
ADOLPHE BOHN.